# EUROPEAN PATENT SPECIFICATION

(11) **EP 3 047 925 B1**
(45) Date of publication and mention of the grant of the patent: **13.04.2022**
(21) Application number: 14845712.0
(22) Date of filing: 17.09.2014
(51) Int. Cl.: B22F 1/00, B22F 7/06, B24C 1/00, B22F 9/04, B02C 19/06, B01J 3/08, C21D 8/02

(54) **SURFACE TREATMENT METHOD FOR POWDERED METAL MATERIAL**
OBERFLÄCHENBEHANDLUNGSVERFAHREN FÜR PULVERFÖRMIGES METALLMATERIAL
PROCÉDÉ DE TRAITEMENT DE SURFACE POUR MATÉRIAU MÉTALLIQUE EN POUDRE

(30) Priority: 18.09.2013 JP 2013193254
(43) Date of publication of application: 27.07.2016
(73) Proprietor: FUJI KIHAN CO., LTD., Aichi 462-0063 (JP)
(72) Inventor: MIYASAKA, Yoshio, Nagoya-shi Aichi 462-0063 (JP)
(74) Representative: Fritz, Edmund Lothar
(86) International application number: PCT/JP2014/074518
(87) International publication number: WO 2015/041236

(56) References cited:
- EP-A1- 0 687 739
- JP-A- H02 243 701
- JP-A- S63 312 071
- JP-A- 2001 225 270
- JP-A- 2007 297 651
- MASATO ISHIWATA: 'Improvement of Metal Surface Strength by Fine Particle Bombarding Treatment' MARINE ENGINEERING vol. 46, no. 5, 01 September 2011, pages 684 - 687, XP055327553

## Description

### FIELD OF THE INVENTION

The present invention relates to a method for surface treatment of a powdery metal material used as a material in manufacture of a metal product or in formation of coating using metal powder such as powder metallurgy such as sintering or thermal spraying.

### DESCRIPTION OF THE RELATED ARTS

The "sintering", i.e., obtaining sintered metal by heating and solidifying an aggregate of a powdery metal material at a temperature lower than a melting point is widely used as a type of powder metallurgy for manufacturing various mechanical components such as gears, and particularly recently, use of the powdery metal material as a shaping material in a 3D printer is proposed. It is also proposed that molding of a desired three-dimensional cubic model directly by the metal material from shape data such as CAD by irradiating a laser beam or an electron beam to a powdery metal material in a predetermined pattern and then sintering it (Non-Patent Document 1), and in the three-dimensional cubic model manufactured by sintering of the powdery metal material as above, unlike a resin model which has been manufactured by a prior-art 3D printer, application not only as a model or a sample but also a direct use as components to be incorporated in a machine or the like are expected.

However, sintered metal obtained by sintering the powdery metal material can easily have a density and strength lower than a case of melt molding due to occurrence of residual pores and the like, and it cannot be used in practice as a mechanical component as it is in many cases.

Thus, with the purpose of removing such residual pores leading to lower density and lower strength, treatment called "sinter forging" for forging the obtained sintered metal has been in practice, but as described above, if treatment of sinter forging is further required for a component manufactured by simple three-dimensional shaping using the 3D printer, the merit of simplicity is lost.

Unlike the post-treatment as the aforementioned sinter forging, researches for improving strength of the sintered metal by devising a composition or structure of the powdery metal material which is a raw material used for sintering have been promoted, and as one of them, there was a report that by applying mechanical milling treatment by stirring with a ball mill to the powdery metal material before sintering so as to change an internal structure of the material, sintered metal with high strength can be obtained (Non-Patent Documents 2 and 3).

In this method, the mechanical milling treatment by a ball mill is performed to the powdery metal material having a predetermined crystalline structure as illustrated in Fig. 6A so as to apply severe plastic deformation to the powdery metal material in a concentrated manner, a region called a shell formed by refining crystal grains (hereinafter this region shall be referred to as a "fine grain region" ) is generated in the vicinity of a surface of the powdery metal material as illustrated in Fig. 6B, and as a result, a powdery metal material can be obtained provided with a region at a center part called a core maintaining an original crystal grain diameter (hereinafter this region shall be referred to as a "coarse grain region") and the aforementioned fine grain region covering this coarse grain region.

By sintering the powdery metal material in which the coarse grain region and the fine grain region are formed as described above, the obtained sintered metal is metal having a structure called "harmonic structure" in which a network-state structure formed of the fine grain regions of the powdery metal materials connected to each other and the coarse grain regions arranged harmonically in the fine grain regions as illustrated in Fig. 6C (in the present invention, such metal is called "harmonic structure metal") is obtained, and it has been reported that in such harmonic structure metal, strength can be drastically improved while ductility equal to that of sintered metal having uniform equiaxed grain structure obtained by using a normal powdery metal material to which the mechanical milling treatment is not applied is maintained (Non-Patent Document 2).

In the aforementioned description, the example in which the manufacturing method of the "harmonic structure metal" is realized by "sintering" is described, but with regard to the powdery metal material provided with the aforementioned fine grain region, the formed metal coating can also be made the "harmonic structure metal" even if the metal coating is formed on the surface of a base material by "thermal spraying".

### DOCUMENTS OF RELATED ART

### NON-PATENT DOCUMENTS

Non-Patent Document 1: "Special Feature 2-3D Printer 'Attracting!' 'Design/Manufacture Solution Exhibition' Report, Diversification of Molding Materials" [issued by Nikkei BP, "Nikkei Monodukuri August issue", (published on August 1, 2013) pp. 64 to 58]
Non-Patent Document 2: "Creation of Innovative Structural Material Realizing both High Strength and High Ductility by Harmonic Structure Control" by Kei Ameyama, Tatsuya Sekiguchi ["Journals of The Japan Society for Heat Treatment" Vol. 53, No. 1 2013" issued by The Japan Society for Heat Treatment (published on February 28, 2013) pp. 1 to 2]
Non-Patent Document 3: "Tripled Renewed Brass Hardness, Chip Molding/Sintering, New Technology by Nihon Univ. Improved Conductivity to Practice" [Nikkan Kogyo Shimbun (April 30, 2013)]
EP 0 687 739 A1 discloses a process to treat the surface of a metal powder material.

### DISCLOSURE OF THE INVENTION

### PROBLEM TO BE SOLVED BY THE INVENTION

As introduced as Non-Patent Documents 2 and 3, when sintering is to be performed by using the powdery metal material subjected to stirring by a ball mill in advance, the sintered metal obtained by the sintering has the "harmonic structure" so that metal having excellent characteristics of both high ductility and high strength is obtained.

However, as described in Non-Patent Documents 2 and 3, when the powdery metal material is treated by the ball mill, treatment efficiency is extremely poor, and treatment time is 100 hours in Non-Patent Document 2 and 32 hours in Non-Patent Document 3 as examples.

Moreover, the treatment of the powdery metal material by the ball mill has a risk of powder dust explosion and is an extremely dangerous work.

That is, since the powdery metal material used for sintering and the like has a fine grain diameter at approximately 100 µm in general, if the powdery metal material is contained in the ball mill, stirred under presence of air and subject to a friction force or an impact force, discharge of static electricity generated by friction in stirring can cause powder dust explosion.

The powder dust explosion here occurs when the following three elements: presence of oxygen; generation of dusts at explosion lower limit density or more; and presence of ignition source are all satisfied and thus, if occurrence of the powder dust explosion is to be prevented, one or more of these conditions need to be eliminated. However, it is impossible to remove occurrence of friction or impact, which can be the ignition source, from the ball mill inside which the friction force and the impact force are generated in order to apply severe plastic deformation to the powdery metal material.

Thus, if the powder dust explosion is to be prevented, the work should be performed in a state in which oxygen is eliminated by filling an inside of the ball mill with an inactive gas or the like, or an input amount of the powdery metal material should be adjusted so as to be less than the explosion lower limit density, or the both should be done.

However, if the treatment is performed in a state in which the ball mill is filled with the inactive gas, a manufacturing cost is drastically raised, and considering that the explosion lower limit density of the powdery metal [200 mesh (opening: 74 µm) completely through] is 35 g/m³ for aluminum, 45 g/m³ for titanium, and 120 g/m³ for iron ["Safety and Hygiene of Arc Welding (third)" extracted from WE-COM magazine No. 6 (published in October 2012), Japan Welding Engineering Society, General Incorporated Association], if stirring is to be performed at the explosion lower limit density or less, only an extremely small amount can be treated at one time. Treatment might be possible for small-scaled production at an experimental level in a lab, but treatment of a large amount of the powdery metal material by a ball mill on a commercial base is impossible.

Moreover, even if the aforementioned treatment by the ball mill can be applied to the treatment of the powdery metal material, surface oxides such as oxidized scale exfoliated from a surface of the powdery metal material are mixed in the powdery metal material treated by this method, and the oxides prevent binding between powdery metal materials during sintering and hinder improvement of strength.

That is, the powdery metal material used for sintering or thermal spraying is manufactured by an atomizing method in general, but since in this atomizing method, the powdery metal material is manufactured by spraying/scattering molten metal for refining and by instantaneously rapid cooling/solidifying it, the oxidized scale adheres to the surface of the powdery metal material.

On the powdery metal materials manufactured by methods other than the atomizing method, an oxidized film which is a surface oxide is also formed more or less by contact with oxygen in the air.

Even if these surface oxides such as the oxidized scale are exfoliated from the surface of the powdery metal material by friction or impact received during stirring in the ball mill, the oxides exfoliated as above are not eliminated even after the exfoliation but stay mixed in the powdery metal material due to a structure of the ball mill.

Moreover, since the exfoliated oxides are continuously stirred together with the powdery metal material in the ball mill, a part of the exfoliated oxides is pressed onto the surface of the powdery metal material by friction or impact caused by stirring and adheres thereto again by being embedded or the like.

Thus, if the powdery metal material treated by the ball mill is taken out as it is and used for sintering, improvement of strength is suppressed by presence of the oxides mixed in the powdery metal material.

On the other hand, in order to remove the oxides mixed in the powdery metal material, the powdery metal material after the treatment by the ball mill can be subjected to wind-power sorting or the like, for example, but with this method, another process for further eliminating the oxides needs to be provided in addition to the treatment by the ball mill, whereby productivity is further lowered.

Moreover, with this method, though the oxides mixed in the powdery metal material can be removed to some degree, the oxides re-adhering to the surface of the powdery metal material cannot be separated/removed.

Thus, if surface treatment of the powdery metal material can be performed by a method which can also remove such surface oxidized film, further improvement of strength of the obtained harmonic structure metal can be expected.

The present invention was made in order to overcome the disadvantages in the aforementioned prior-art techniques and has an object to provide a method defined by the appended claim 1 without a concern of powder dust explosion and can perform exfoliation of oxides from the surface and removal of the oxides after the exfoliation easily and reliably and also efficiently in a relatively short time.

### MEANS FOR SOLVING THE PROBLEMS

In order to achieve an objective of the invention, a method for surface treatment of a powdery metal material for manufacture of harmonic structure metal in which a fine grain region and a coarse grain region are harmonically is defined by the appended claim 1.

Furthermore, in the dust collecting means of the blasting machine, the collected powder dusts are stored with nonflammable powder, such as calcium carbonate or the like.

In the method for surface treatment of a powdery metal material, the ejection powder and the object to be collided may be exchanged each other, i.e., the blasting may be performed by using the powdery metal material as the ejection powder and the medium substance as the object to be collided; and
the blasting may be performed by using the medium substance with a powdery shape as the ejection powder and the powdery metal material as the object to be collided.

Furthermore, the medium substance may be made a powdery metal material of the same material and the same average grain diameter as the powdery metal material, and the ejection powder and the object to be collided may be both made into the powdery metal material.

A material of the medium substance may be metal having hardness equal to or higher than hardness of the powdery metal material or ceramic having hardness equal to or higher than hardness of the powdery metal material after the surface treatment.

### EFFECT OF THE INVENTION

According to the method for surface treatment of the powdery metal material of the present invention, the following marked effects can be obtained by means of the aforementioned constitution of the present invention.

By performing blasting of causing a powdery metal material having an average grain diameter of 10 to 200 µm and a medium substance having hardness equal to or higher than that of the powdery metal material to be collided with each other repeatedly at an ejection speed of 100 to 300 m/sec, surface oxides on the powdery metal material are removed, and repetition of rapid temperature rise and cooling occurring in the vicinity of a surface of the powdery metal material at the collision refines crystal grains in the vicinity of the surface of the powdery metal material, and the powdery metal material in which a fine grain region having a crystal grain diameter smaller than a crystal grain diameter at a center part is formed in the vicinity of the surface can be treated by a relatively simple method of blasting easily and in a large quantity in a short time.

Moreover, by performing the aforementioned blasting by means of a blasting machine with a dust collection function, mass production is made possible while a risk of powder dust explosion is avoided, and by removing and collecting surface oxides such as oxidized scale exfoliated from the surface of the powdery metal material as powder dusts by suctioning in a cabinet, a powdery metal material without mixing of the surface oxides could be obtained without separately providing a process of removing the surface oxides in a post-process.

The means provided with a cyclone for classifying the powder dusts from the ejected powder is to be used as dust collecting means for the blasting, even if the powdery metal powder and the exfoliated surface oxides are collected in the mixed state, the surface oxides can be classified with the powder dusts from the ejected powder and collected so that the powdery metal material from which the surface oxides are removed with higher accuracy could be obtained.

Moreover, in the dust collecting means of the aforementioned blasting machine, if the removed powder dusts are stored with nonflammable powder such as calcium carbonate, a risk of powder dust explosion not only in a processing chamber but also in the collecting machine could be reduced.

This blasting may be so configured that the powdery metal material as the ejection powder is ejected to the medium substance and made to collide against said medium substance, or that the medium substance as the ejection powder is ejected to the powdery metal material and is made to collide against said powdery metal material, but when it is so configured that both the ejection powder and an object to be collided are made to be a powdery metal material having the same average grain diameter and formed of the same material and the powdery metal material is ejected to and is made to collide against the powdery metal material, the surface treatment is applied to both the powdery metal powder as the ejection powder and the powdery metal powder as the object to be collided, and a throughput could be doubled.

### BRIEF DESCRIPTION OF THE DRAWINGS

Fig. 1A is schematic explanatory view of a blasting machine of a gravity type used in a method for surface treatment of the present invention;
Fig. 1B is schematic explanatory view of a blasting machine of a direct pressure type used in a method for surface treatment of the present invention;
Fig. 2 is a graph showing an X-ray diffraction result of an untreated stainless powder (SUS304 equivalent);
Fig. 3 is a graph showing an X-ray diffraction result of a stainless powder (SUS 304 equivalent) treated by a method in Example 1;
Fig. 4 is a graph showing an X-ray diffraction result of an untreated powder high-speed tool steel (SKH equivalent);
Fig. 5 is a graph showing an X-ray diffraction result of a powder high-speed tool steel (SKH equivalent) treated by a method in Example 2; and
Fig. 6A is an explanatory view explaining creation of a harmonic structure in which is a schematic view of an untreated powdery metal material;
Fig. 6B is an explanatory view explaining creation of a harmonic structure in which is a schematic view of a powdery metal material after treatment by a ball mill; and
Fig. 6C is an explanatory view explaining creation of a harmonic structure in which is a schematic view of harmonic structure metal obtained by sintering the powdery metal material in Fig. 6B.

Subsequently, embodiments of the present invention will be described below by referring to the attached drawings.

### ENTIRE CONFIGURATION

The present invention is to remove surface oxides such as an oxidized scale prohibiting improvement of strength in sintering or thermal spraying from a surface of a powdery metal material and to form a fine grain region having a crystal grain diameter smaller than the crystal grain diameter at a center part in the vicinity of the surface of the powdery metal material by performing blasting of repeatedly causing the powdery metal material which is a treatment target and a medium substance which collides against the powdery metal material to collide against each other at a predetermined ejection speed by means of a known blasting machine.

As described above, a metal product obtained by a method of powder metallurgy such as sintering or metal coating manufactured by thermal spraying by using a powdery metal material in which a coarse grain region having a relatively large crystal grain diameter is formed at the center part and a fine grain region with a smaller crystal grain diameter than that of the coarse grain region is formed in the vicinity of the surface become harmonic structure metal having a crystalline structure [see Fig. 6C] in which the coarse grain regions are harmonically arranged in a network of a fine grain structure formed by binding the fine grain regions and exhibiting an excellent characteristic that both high ductility and high strength are realized.

### POWDERY METAL MATERIAL

The powdery metal material which is a treatment target in the present invention is powdery metal having an average grain diameter of 10 to 200 µm to be used as a material in powder metallurgy as sintering or thermal spraying, and various materials can be used as long as it is applicable to powder metallurgy or thermal spraying. The material may be constituted by either one of pure metal and an alloy.

As an example, metal used for powder metallurgy in general includes iron-, copper-, stainless-, titanium-, and tungsten-based metal and metal used for thermal spraying in general includes zinc, aluminum, copper and the like. They can be all included in the material of the powdery metal material in the present invention.

The powdery metal material to be used can be manufactured by various methods, e.g. spraying methods represented by an atomizing method which is a manufacturing method of the powdery metal material used in general in the powder metallurgy and thermal spraying, and various known methods such as mechanical crushing, electrolytic deposition and the like.

A shape of the powder may be spherical but this is not limiting and those with various shapes can be used.

The crystal grain diameter of the powdery metal material before treatment is a crystal grain diameter of the aforementioned coarse grain region as it is, and if the crystal grain diameter of the coarse grain region is set within a predetermined range, a powdery metal material with a corresponding crystal grain diameter is selected. Though not particularly limiting, the average crystal grain diameter of the coarse grain region is several to several tens µm as an example.

### MEDIUM SUBSTANCE

As the aforementioned medium substance which collides against the powdery metal material, various substances can be used as long as it has hardness equal to or higher than that of the powdery metal material, and not only those made of metal but those made of ceramic can be used.

If the medium substance made of ceramic not subjected to work hardening is to be used, it is preferable that ceramic having hardness equal to or higher than that of the powdery metal material after the surface treatment of the present invention is used so that the powdery metal material can maintain the same or improved hardness after the work hardening.

By constituting the medium substance itself by the aforementioned powdery metal material, the aforementioned fine grain region may be formed in the both of the powdery metal material as the treatment target and the powdery metal material as the medium substance by collision between the powdery metal materials.

A shape of the medium substance needs to be constituted as powder when the medium substance is to be used as the ejection powder, but when the treatment is to be performed by using the aforementioned powdery metal material as the ejection powder, the medium substance does not have to be powder but may be constituted in a form of a plate body or the like.

### BLASTING METHOD AND BLASTING MACHINE

The collision between the powdery metal material and the medium substance described above is made by blasting means of the blasting machine.

As this blasting, as described above, it may be so configured that the powdery metal material is ejected as the ejection powder to the medium substance and made to collide against said medium substance, or to the contrary, a powdery medium substance may be prepared as the ejection powder and ejected to the powdery metal material so as to cause a collision against said powdery metal material. Moreover, it may be so configured that the ejection powder and the object to be collided are both constituted by the powdery metal material having the same average grain diameter and made of the same material, and the powdery metal materials are made to collide against each other.

As the blasting machine 1 to be used, those with various known constitution can be used as long as it is a blasting machine having a cabinet 21 as a processing chamber and a dust collection function of suctioning an inside of the cabinet 21 for dust collection, and the blasting machine of either one of a direct pressure type and a gravity type may be used.

A constitution example of the gravity type blasting machine 1 and a constitution example of the direct pressure type to be used for the surface treatment of the present invention are illustrated in Fig. 1A and Fig. 1B, respectively.

An example in which the surface treatment of the present invention is performed with the blasting machine 1 by using the powdery metal material having the same material and the same average grain diameter for both the ejection powder and the object to be collided will be described below. However, the blasting machine 1 used in the method for surface treatment of the present invention is not limited to illustrated constitution.

The blasting machine 1 illustrated in Figs. 1A and 1B comprises: the cabinet 21 which becomes a processing chamber for accommodating an ejection nozzle 22 and a workpiece and performing blasting; and a dust collecting machine 38 for suctioning an inside of this cabinet 21. The blasting machine 1 is provided with a cyclone type collection tank 23 between this dust collecting machine 38 and the cabinet 21 for collecting into the collection tank 23 the powdery metal material collected by suctioning of the inside of the cabinet 21 in a state mixed with powder dusts and can collect into the dust collecting machine 38 the powder dusts separated from the powdery metal material in the cyclone type collection tank 23.

It is configured that the powdery metal material collected in the collection tank 23 as described above can be ejected again by an ejection nozzle 22 in the cabinet 21.

At a destination to which a tip end of the ejection nozzle 22 is directed inside the aforementioned cabinet 21, a barrel basket 24 which is a container rotating during ejection of the ejection powder and opened upward is provided, and the powdery metal material which is the object to be collided can be input therein.

In the example illustrated in Fig. 1A, this barrel basket 24 is depicted as a mesh with a large number of small pores formed, but the illustrated example is not limiting, and the barrel basket may be constituted without such small pores.

Prior to the treatment by means of the blasting machine 1 constituted as above, the powdery metal material is contained in the collection tank 23 and the powdery metal material is also contained in the barrel basket 24 provided in the processing chamber, and while the barrel basket 24 is rotated in this state, ejection of the powdery metal material from the ejection nozzle 22 is started at the ejection speed of 100 to 300 m/sec and then, the powdery metal material ejected from the ejection nozzle 22 collides against the powdery metal material in the rotating barrel basket 24.

An ejection pressure may be 100 m/sec or more in the treatment of a non-iron based powdery metal material, but 150 m/sec or more is preferable for the treatment of an iron-based powdery metal material.

By performing ejection of the powdery metal material as described above, the powdery metal material in the barrel basket 24 and the powdery metal material ejected from the ejection nozzle 22 mutually receive energy at the collision so that surface oxides such as oxidized scale formed on the surface of the powdery metal materials are exfoliated. Also, the temperature of the surface in the collision portion is rapidly raised and also cooled so that the crystal grains on the surface of the collision portion are refined, and a fine grain region is formed in which a crystal grain with a diameter smaller than that of the crystal grain on a center portion of the powdery metal material is formed in the vicinity of the surface of the powdery metal material.

It is empirically confirmed that the fine grain region of the powdery metal material is formed on the surface of the powdery metal material to a depth of approximately 20% at the maximum with respect to the grain diameter if the powdery metal material as the treatment target is less than 100 µm and formed to a depth of approximately 10% at the maximum with respect to the grain diameter if the powdery metal material as the treatment target is 100 µm or more, and thus, in the method for surface treatment of the present invention with the powdery metal material having an average grain diameter of 10 to 200 µm as the treatment target, the aforementioned fine grain region is formed within a range of 2 to 20 µm from the surface at the maximum depending on the grain diameter of the powdery metal material as the treatment target.

A description "in the vicinity of the surface" used herein refers to the surface including the above described range of depth.

The powdery metal material ejected from the ejection nozzle 22 collides against the powdery metal material in the barrel basket 24 and then, accumulates in the barrel basket 24 except those forced out to outside the barrel basket 24 and is stirred with rotation of the barrel basket 24 with the powdery metal material having been originally present in the barrel basket 24.

Thus, if the ejection of the powdery metal material from the ejection nozzle 22 is continued, the powdery metal material in the barrel basket 24 increases and overflows from the barrel basket 24 and drops to a bottom part of the cabinet 21.

The bottom part of the cabinet 21 is formed as a hopper having an inverted trapezoidal shape, and a lower end of the hopper communicates with the dust collecting machine 38 through an exhaust air passage 33 and the collection tank 23 and thus, when the inside of the cabinet 21 is suctioned by a ventilator 39 provided in the dust collecting machine 38, the dropped powdery metal material and powder dusts are suctioned with the air in the cabinet 21 and supplied into the cyclone type collection tank 23, the powder dusts and the powdery metal material are classified in this collection tank 23 and the powdery metal material is collected downward in the collection tank 23.

The surface oxides such as oxidized scale generated on the surface of the powdery metal material are harder and more fragile as compared with the powdery metal material. Therefore, the surface oxides are finely crushed when they are exfoliated by an impact caused by a collision between the powdery metal materials. Thus, the surface oxides are not collected in the collection tank 23 but sent to the dust collecting machine 38 as powder dusts through a pipe 32 connected to an upper part of the collection tank 23 and collected downward in the dust collecting machine 38, and clean air is discharged to the outside air by the ventilator 39.

As described above, the inside of the processing chamber formed in the cabinet 21 is suctioned at all times, and the powder dusts and the powdery metal material floating in the air are removed and kept to the explosion lower limit density or less. Thus, there is no concern of the powder dust explosion in the cabinet even by heat generation by ejection, collision and friction of the ejection powder which is the powdery metal material or generation of static electricity in this embodiment.

On the other hand, the powder dusts classified in the cyclone type collection tank 23 and collected in the dust collecting machine 38 are accommodated in the dust collecting machine 38 with an nonflammable powder such as powder of calcium carbonate, for example, so that a density of flammable powder dusts in the air in the dust collecting machine 38 becomes the explosion lower limit density or less, whereby a risk of powder dust explosion in the dust collecting machine 38 is also avoided.

The powdery metal material collected in the collection tank 23 is ejected again by the ejection nozzle 22 toward the powdery metal material in the barrel basket 24, and the aforementioned process is repeated so that the surface oxides such as oxidized scale are removed from the surfaces of any powdery metal materials, and the fine grain region is formed so as to cover the entirety in the vicinity of the surface.

When the powdery metal material on which the fine grain region is formed in the vicinity of the surface as described above is used as a material for powder metallurgy such as sintering or is used for formation of a metal film of thermal spraying or the like, in the obtained sintered metal or metal coating, harmonic structure metal in which the coarse grain region is harmonically arranged in the network of the fine grain structures formed by mutually connecting parts of the fine grain regions is obtained. In such harmonic structure metal, excellent characteristics of realization of both the high ductility and high strength are obtained.

Particularly in the powdery metal material treated by the method of the present invention, the surface oxides such as oxidized scale causing lowered strength in sintering or deposition can be favorably removed and thus, strength of the obtained sintered metal or metal coating can be further improved.

In the aforementioned description, the constitution is described in which the ejection powder and the object to be collided are both the powdery metal materials and the ejection powder and the object to be collided are made to collide against each other in the barrel basket 24 provided in the cabinet 21, but a plate body formed of a material having hardness equal to or higher than that of the ejection powder is accommodated as the medium substance in the cabinet 21 instead of the aforementioned barrel basket 24, and the surface treatment of the present invention may be configured to be performed by ejecting the powdery metal material as the ejection powder to this plate body and making to collide against the same.

Moreover, it may be so constituted that the aforementioned blasting machine 1 provided with the barrel basket 24 is used, a powdery medium substance is used as the ejection powder, and the medium substance as the ejection powder is ejected to the powdery metal material contained in the barrel basket 24, and in this case, the powdery metal material and the medium substance are classified after the treatment and collected, respectively.

### EXAMPLES

Examples in which the method for surface treatment of the present invention is applied to the powdery metal materials of various materials will be described below.

### EXAMPLE 1

The method for surface treatment of the present invention was performed to stainless powder (SUS304 equivalent: #80) as the powdery metal material. Treatment conditions are shown in Table 1 below:

**TABLE 1**

| Treatment conditions for Example 1 (SUS304) | | |
|---|---|---|
| Blasting machine | Type | Direct pressure type ("FD-4LD" by Fuji Manufacturing Co., Ltd.) |
| | Barrel basket | made of SUS304, no pores, 4 rotations per minute |
| | Nozzle | Nozzle diameter: ϕ5 mm Oscillation: 100 mm in width, 60 times per minute |
| Powdery metal material | Material | Stainless powder (SUS-304 equivalent) (0.2 to 0.3%C <1.8%Si <1.0%Mn 18 to 20%Cr 8 to 10.5%Ni) |
| | Grain diameter | #80 (105 to 250µm / 177µm on average) |
| Medium substance | | Same as powdery metal material |
| Blasting conditions | Ejection pressure | 0.6 MPa |
| | Ejection speed | 150m/sec or more |
| | Ejection distance | 300 mm |
| | Ejection rate | 6 kg/min |
| | Ejection time | 3 hours |
| | Throughput | 30 kg |

The stainless powder in 10 kg was contained in the barrel basket provided in the processing chamber of the blasting machine and 20 kg into the collection tank, and the treatment of ejecting the stainless powder in the collection tank by the ejection nozzle into the barrel basket was performed continuously for 3 hours under the condition shown in the aforementioned Table 1.

As the result of the aforementioned treatment, in the stainless powder after the treatment, the oxidized scale was removed and the surface was cleaned, and moreover, hardness of the stainless powder which was 250 to 350 HV before the treatment rose to 450 to 550 HV after the treatment, and it is expected from the result that the crystal grains in the vicinity of the surface were refined.

Refining of the crystal grain diameter can be evaluated from an increase of a line width of an X-ray analysis peak using the Scherrer (Sherrer, 1918) formula. In the X-ray analysis result (Fig. 3) after the treatment by the present invention, the line width of the peak drastically increased with respect to the X-ray analysis result (see Fig. 2) of the untreated stainless powder. Thus, it was confirmed that hardness of the aforementioned powdery metal material rose, and refining of the crystal grain diameter on the surface was also confirmed from the X-ray diffraction result.

### EXAMPLE 2

The method for surface treatment of the present invention was performed to a powder high-speed tool steel (SKH equivalent: #150) as the powdery metal material. The treatment conditions are shown in Table 2 below:

**TABLE 2**

| Treatment conditions for Example 2 (Powder high-speed tool steel: SKH equivalent) | | |
|---|---|---|
| Blasting machine | Type | Gravity type ("SGK-4LD" by Fuji Manufacturing Co., Ltd.) |
| | Barrel basket | made of SUS304, no pores, 4 rotations per minute |
| | Nozzle | Nozzle diameter: ϕ9 mm Oscillation: 100 mm in width, 60 times per minute |
| Powdery metal material | Material | Powder high-speed tool steel ("SPM30" by Sanyo Special Steel Co., Ltd.) (1.3%C 4.0%Cr 5%Mo 6%W 3%V 8%Co) |
| | Grain diameter | #150 (44 to 125µm / 85µm on average) |
| Medium substance | | Same as powdery metal material |
| Blasting conditions | Ejection pressure | 0.6 MPa |
| | Ejection speed | 150m/sec or more |
| | Ejection distance | 200 mm |
| | Ejection rate | 5 kg/min |
| | Ejection time | 5 hours |
| | Throughput | 20 kg |

The powdery high-speed tool steel in 10 kg was contained in the barrel basket provided in the processing chamber of the blasting machine and 10 kg into the collection tank, and the treatment of ejecting the powdery high-speed tool steel in the collection tank by the ejection nozzle into the barrel basket was performed continuously for 5 hours under the conditions shown in the aforementioned Table 2.

As a result, hardness of the powdery high-speed tool steel at 650 to 750 HV before the treatment rose to 900 to 1000 HV after the treatment.

Moreover, in the powdery high-speed tool steel after the treatment, the oxidized scale was removed and the surface was cleaned, and from the X-ray diffraction result, the line width of the X-ray analysis peak increased (see Fig. 5) as compared with the untreated one (see Fig. 4), and the refining of the surface structure by the treatment according to the method of the present invention was confirmed (see Figs. 4 and 5).

### EXAMPLE 3

The method for surface treatment of the present invention was performed to powder of an alloy steel for mechanical structure (SCM equivalent: #150) as the powdery metal material. The treatment conditions are shown in Table 3 below:

**TABLE 3**

| Example 3: Treatment conditions for powder of alloy steel for mechanical structure (SCM equivalent) | | |
|---|---|---|
| Blasting machine | Type | Gravity type ("SGK-4LD" by Fuji Manufacturing Co., Ltd.) |
| | Barrel basket | made of SUS304, no pores, 4 rotations per minute |
| | Nozzle | Nozzle diameter: ϕ9 mm Oscillation: 100 mm in width, 60 times per minute |
| Powdery metal material | Material | Alloy steel for mechanical structure (SCM equivalent) (0.23%C 0.2%Mo 1.5%Cr) |
| | Grain diameter | #150(44 to 125µm / 85µm on average) |
| Medium substance | | Same as powdery metal material |
| Blasting conditions | Ejection pressure | 0.6 MPa |
| | Ejection speed | 150 m/sec or more |
| | Ejection distance | 200 mm |
| | Ejection rate | 5 kg/min |
| | Ejection time | 5 hours |
| | Throughput | 20 kg |

The power of alloy steel for mechanical structure in 10 kg was contained in the barrel basket provided in the processing chamber of the blasting machine and 10 kg into the collection tank, and the treatment of ejecting the powder of the alloy steel for mechanical structure in the collection tank by the ejection nozzle into the barrel basket was performed continuously for 5 hours under the conditions shown in the aforementioned Table 3.

As a result, hardness of the powder of alloy steel for mechanical structure at 150 to 200 HV before the treatment rose to 300 to 350 HV after the treatment.

Moreover, in the powder of the alloy steel for mechanical structure after the treatment, the oxidized scale was removed and the surface was cleaned, and it is considered from the aforementioned rise of hardness that the refined structure is formed on the surface.

### EXAMPLE 4

The method for surface treatment of the present invention was performed to powder of the copper alloy (#150) as the powdery metal material. The treatment conditions are shown in Table 4 below:

**TABLE 4**

| Treatment conditions for Example 4 (copper alloy) | | |
|---|---|---|
| Blasting machine | Type | Gravity type ("SGK-4LD" by Fuji Manufacturing Co., Ltd.), No barrel basket |
| | Nozzle | Nozzle diameter = ϕ9 mm Oscillation: 100 mm in width, 60 times per minute |
| Powdery metal material | Material | Copper alloy (21%Zn 17%Ni 0.34%Mn, the remnant Cu) |
| | Grain diameter | #150 (44 to 125µm / 85µm on average) |
| Medium substance | | SKD11 plate having diameter of 400 mm and thickness of 20 mm |
| Blasting conditions | Ejection pressure | 0.4 MPa |
| | Ejection speed | 100m/sec or more |
| | Ejection distance | 200 mm |
| | Ejection rate | 4 kg/min |
| | Ejection time | 7 hours |
| | Throughput | 20 kg |

The copper alloy powder in 20 kg was contained in the collection tank, and the treatment of ejecting the copper alloy powder in the collection tank by the ejection nozzle toward a position where a core was shifted by 100 mm from a center of a plate (φ400 mm, thickness 20 mm) made of SKD11 arranged in the processing chamber was performed for 7 hours continuously.

As a result, hardness of the copper alloy powder at 160 to 200 HV before the treatment rose to 220 to 260 HV after the treatment.

Moreover, in the copper alloy powder after the treatment, the oxidized scale was removed and the surface was cleaned, and it is considered from the aforementioned rise of hardness that the refined structure is formed on the surface.

### EXAMPLE 5

The method for surface treatment of the present invention was performed to powder of aluminum alloy (AC8A: #80) as the powdery metal material. The treatment conditions are shown in Table 5 below:

**TABLE 5**

| Treatment conditions for Example 5: Aluminum alloy (AC8A) | | |
|---|---|---|
| Blasting machine | Type | Gravity type ("SGK-4LD" by Fuji Manufacturing Co., Ltd.) |
| | Barrel basket | made of SUS304, with (ϕ1 mm pores, 4 rotations per minute |
| | Nozzle | Nozzle diameter: ϕ9 mm Oscillation: 100 mm in width, 60 times per minute |
| Powdery metal material | Material | Aluminum alloy (AC8A:12%Si 0.8%Fe 1.1%Cu 0.15%Mn 1%Mg 1.1%Ni, the remnant Al) |
| | Grain diameter | #80 (105 to 250µm / 177µm on average) |
| Medium substance | | Shot made of a high speed steel (#400, 45µm on average) |
| Blasting conditions | Ejection pressure | 0.4 MPa |
| | Ejection speed | 100 m/sec or more |
| | Ejection distance | 200 mm |
| | Ejection rate | 4 kg/min |
| | Ejection time | 7 hours |
| | Throughput | 10 kg |

A barrel basket in which a large number of holes, each having a diameter of 1 mm, are formed was provided in the processing chamber, and the powder of the aluminum alloy (AC8A) was input in 10 kg into this barrel basket, and a treatment of ejecting a shot made of a high speed steel collected in the collection tank into the barrel basket was performed for 7 hours continuously.

As a result of the aforementioned treatment, hardness of the aluminum alloy powder at 120 to 140 HV before the treatment rose to 200 to 250 HV after the treatment.

Moreover, in the aluminum alloy powder after the treatment, the oxidized scale was removed and the surface was cleaned, and from the aforementioned rise of hardness, it is considered that a component of the high speed steel which is the medium substance is diffused and penetrated into the surface of the powder of the aluminum alloy and the refined structure was formed on the surface.

### SINTERING TEST RESULT

Then, discharge plasma sintering was performed by using the powdery metal material treated by the method for surface treatment of the present invention described as above as Examples 1 to 5.

As a result, also in the sintered metal obtained by sintering the powdery metal material of any one of examples 1 to 5, the "harmonic structure" in which the coarse grain structures are arranged harmonically in the network formed by connecting the fine grain regions to each other is provided, and it was confirmed that the method for surface treatment of the present invention is a method for surface treatment which can treat the powdery metal material used for manufacture of the harmonic structure metal simply, in a large quantity and moreover, safely.

### Descriptions of Reference Numerals

- 1.: Blasting machine
- 21.: Cabinet
- 22.: Ejection nozzle
- 23.: Collection tank (cyclone type)
- 24.: Barrel basket
- 32.: Pipe
- 33.: Exhaust air passage
- 38.: Dust collecting machine
- 39.: Ventilator

## Claims

1. A method for surface treatment of a powdery metal material for manufacturing a harmonic structure metal in which a fine grain region and a coarse grain region are harmonically arranged comprising the steps of:
ejecting ejection powder with a compressed gas in a cabinet by use of a blasting machine and causing the ejection powder to collide against an object to be collided, suctioning an inside of the cabinet by dust collecting means and removing/collecting powder dusts, namely surface oxides such as oxidized scale exfoliated from the surface of the powdery metal material; and
performing blasting by causing a powdery metal material having an average grain diameter of 10 to 200 µm and a medium substance having hardness equal to or higher than that of the powdery metal material to collide with each other repeatedly at an ejection speed of 100 to 300 m/sec, and exfoliate surface oxides from the powdery metal material and forming a fine grain region called a shell in the vicinity of the surface of the powdery material and a region at a center part called a core maintaining an original crystal grain diameter, the fine grain region covering this coarse grain region,
wherein the fine grain region which is formed in the vicinity of the surface of the powdery metal material has a crystal grain with a diameter smaller than that of the crystal grain on a center portion of the powdery metal material which is formed, wherein the fine grain region of the powdery metal material is formed on the surface of the powdery metal material to a depth of approximately 20% at the maximum with respect to the grain diameter if the powdery metal material as the treatment target is less than 100 µm and formed to a depth of approximately 10% at the maximum with respect to the grain diameter if the powdery metal material as the treatment target is 100 µm or more,
sintering the powdery material or using the powdery material for formation of a metal film by thermal spraying, and obtaining a network-state structure formed of the fine grain regions of the powdery metal materials connected to each other and the coarse grain regions arranged harmonically in the fine grain regions.

2. The method for surface treatment of a powdery metal material according to claim 1, wherein
the dust collecting means of the blasting machine comprises a cyclone for classifying the powder dusts and the ejection powder.

3. The method for surface treatment of a powdery metal material according to claim 1 or 2, wherein
in the dust collecting means of the blasting machine, the collected powder dusts are stored with nonflammable powder.

4. The method for surface treatment of a powdery metal material according to any one of claims 1 to 3, wherein
the blasting is performed by using the powdery metal material as the ejection powder and the medium substance as the object to be collided.

5. The method for surface treatment of a powdery metal material according to any one of claims 1 to 3, wherein
the blasting is performed by using the medium substance with a powdery shape as the ejection powder and the powdery metal material as the object to be collided.

6. The method for surface treatment of a powdery metal material according to any one of claims 1 to 3, wherein
the medium substance is made a powdery metal material of the same material and the same average grain diameter as the powdery metal material, and the ejection powder and the object to be collided are both made into the powdery metal material.

7. The method for surface treatment of a powdery metal material according to any one of claims 1 to 5, wherein
a material of the medium substance is metal having hardness equal to or higher than hardness of the powdery metal material or ceramic having hardness equal to or higher than hardness of the powdery metal material after the surface treatment.

## Patentansprüche

1. Verfahren zur Oberflächenbehandlung eines pulverförmigen Metallmaterials zur Herstellung eines Metalls mit harmonischer Struktur, in dem ein feinkörniger Bereich und ein grobkörniger Bereich harmonisch angeordnet sind, das die folgenden Schritte umfasst:
Ausstoßen von Ausstoßpulver mit einem komprimierten Gas in ein Behältnis unter Verwendung einer Strahlvorrichtung und Bewirken, dass das Ausstoßpulver auf ein zu treffendes Objekt prallt, Absaugung des Innenraums des Behältnisses durch ein Staubauffangsystem und Entfernen/Auffangen von Feinstäuben, nämlich von Oberflächenoxiden, wie oxidiertem Zunder, der sich von der Oberfläche des pulverförmigen Metallmaterials ablöst; und
Durchführen des Strahlens, indem ein pulverförmiges Metallmaterial mit einem durchschnittlichen Korndurchmesser von 10 bis 200 µm und eine Trägersubstanz mit einer Härte, die höher oder gleich der des pulverförmigen Metallmaterials ist, wiederholt mit einer Ausstoßgeschwindigkeit von 100 bis 300 m/s aufeinander prallen, und Abblättern von Oberflächenoxiden von dem pulverförmigen Metallmaterial und Bilden eines feinkörnigen Bereichs, der als Schale bezeichnet wird, in der Nähe der Oberfläche des pulverförmigen Materials und eines Bereichs in der Mitte, der als Kern bezeichnet wird und einen ursprünglichen Kristallkorndurchmesser beibehält, wobei der feinkörnige Bereich diesen grobkörnigen Bereich bedeckt,
wobei der feinkörnige Bereich, der in der Nähe der Oberfläche des pulverförmigen Metallmaterials gebildet ist, ein Kristallkorn mit einem Durchmesser hat, der kleiner als der des Kristallkorns in einem mittleren Teil des gebildeten pulverförmigen Metallmaterials ist,
wobei der feinkörnige Bereich des pulverförmigen Metallmaterials auf der Oberfläche des pulverförmigen Metallmaterials bis zu einer Tiefe von maximal ca. 20 % bezüglich des Korndurchmessers gebildet ist, wenn das pulverförmige Metallmaterial als Ziel der Behandlung kleiner als 100 µm ist, und bis zu einer Tiefe von maximal ca. 10 % bezüglich des Korndurchmessers gebildet ist, wenn das pulverförmige Metallmaterial als Ziel der Behandlung 100 µm oder mehr ist,
Sintern des pulverförmigen Metallmaterials oder Verwenden des pulverförmigen Metallmaterials zur Bildung eines Metallfilms durch thermisches Spritzen und Gewinnen einer Netzstruktur, die aus den Feinkornbereichen der pulverförmigen Metallmaterialien, welche miteinander verbunden sind, und den grobkörnigen Bereichen, die harmonisch in den Feinkornbereichen angeordnet sind, gebildet sind.

2. Verfahren zur Oberflächenbehandlung eines pulverförmigen Metallmaterials nach Anspruch 1, wobei das Staubauffangsystem der Strahlvorrichtung einen Fliehkraftabscheider zur Klassierung der pulverförmigen Stäube und des Ausstoßpulvers enthält.

3. Verfahren zur Oberflächenbehandlung eines pulverförmigen Metallmaterials nach Anspruch 1 oder 2, wobei im Staubauffangsystem der Strahlvorrichtung die aufgefangenen Stäube mit einem nicht brennbaren Pulver gelagert werden.

4. Verfahren zur Oberflächenbehandlung eines pulverförmigen Metallmaterials nach einem der Ansprüche 1 bis 3, wobei das Strahlen ausgeführt wird unter Verwendung des pulverförmigen Metallmaterials als Ausstoßpulver und der Mittelsubstanz als das zu treffende Objekt.

5. Verfahren zur Oberflächenbehandlung eines pulverförmigen Metallmaterials nach einem der Ansprüche 1 bis 3, wobei das Strahlen ausgeführt wird unter Verwendung der Mittelsubstanz mit einer pulvrigen Form als Ausstoßpulver und das pulverförmige Metallmaterial als das zu treffende Objekt.

6. Verfahren zur Oberflächenbehandlung eines pulverförmigen Metallmaterials nach einem der Ansprüche 1 bis 3, wobei die Mittelsubstanz zu einem pulverförmigen Metallmaterial desselben Materials und mit demselben durchschnittlichen Korndurchmesser wie das pulverförmige Metallmaterial gemacht wird, und das Ausstoßpulver und das zu treffende Objekt werden beide zum pulverförmigen Metallmaterial gemacht.

7. Verfahren zur Oberflächenbehandlung eines pulverförmigen Metallmaterials nach einem der Ansprüche 1 bis 5, wobei ein Material der Mittelsubstanz ein Metall ist, das eine Härte hat, die größer oder gleich der Härte des pulverförmigen Metallmaterials ist, oder Keramik mit einer Härte, die größer oder gleich der Härte des pulverförmigen Metallmaterials nach der Oberflächenbehandlung ist.

## Revendications

1. Procédé de traitement de surface d'un matériau métallique pulvérulent pour la fabrication d'un métal à structure harmonique dans lequel une région de grains fins et une région de gros grains sont agencées de manière harmonique, comprenant les étapes consistant à :
éjecter une poudre d'éjection avec un gaz comprimé dans une enceinte par utilisation d'une machine de grenaillage et provoquer la collision de la poudre d'éjection contre un objet à heurter, aspirer un intérieur de l'enceinte à l'aide d'un moyen de collecte de poussière et retirer/collecter les poussières d'énergie, à savoir les oxydes de surface tels que le tartre oxydé exfolié de la surface du matériau métallique pulvérulent ; et
effectuer un grenaillage en provoquant la collision d'un matériau métallique pulvérulent ayant un diamètre de grain moyen de 10 à 200 µm et d'une substance support ayant une dureté égale ou supérieure à celle du matériau métallique pulvérulent l'un avec l'autre de manière répétée à une vitesse d'éjection de 100 à 300 m/sec, et exfolier les oxydes de surface du matériau métallique pulvérulent et former une région de grains fins, appelée enveloppe, à proximité de la surface du matériau pulvérulent et une région au niveau d'une partie centrale, appelée cœur, maintenant un diamètre de grain cristallin initial, la région de grains fins recouvrant la région de gros grains,
dans lequel la région de grains fins qui est formée à proximité de la surface du matériau métallique pulvérulent a un grain cristallin ayant un diamètre inférieur à celui du grain cristallin sur une partie centrale du matériau métallique pulvérulent qui est formé,
dans lequel la région de grains fins du matériau métallique pulvérulent est formée sur la surface du matériau métallique pulvérulent à une profondeur d'environ 20 % au maximum par rapport au diamètre de grain si le matériau métallique pulvérulent en tant que cible de traitement est inférieur à 100 µm et formée à une profondeur d'environ 10 % au maximum par rapport au diamètre de grain si le matériau métallique pulvérulent en tant que cible de traitement est de 100 µm ou plus,
fritter le matériau pulvérulent ou utiliser le matériau pulvérulent pour la formation d'un film métallique par pulvérisation thermique, et obtenir une structure d'état de réseau se composant des régions de grains fins des matériaux métalliques pulvérulents reliées les unes aux autres et des régions de gros grains disposées de manière harmonique dans les régions de grains fins.

2. Procédé de traitement de surface d'un matériau métallique pulvérulent selon la revendication 1, dans lequel le moyen de collecte de poussière de la machine de grenaillage comprend un cyclone pour classer les poussières d'énergie et la poudre d'éjection.

3. Procédé de traitement de surface d'un matériau métallique pulvérulent selon la revendication 1 ou 2, dans lequel dans le moyen de collecte de poussière de la machine de grenaillage, les poussières d'énergie collectées sont stockées avec de la poudre non inflammable.

4. Procédé de traitement de surface d'un matériau métallique pulvérulent selon l'une quelconque des revendications 1 à 3, dans lequel le grenaillage est effectué en utilisant le matériau métallique pulvérulent comme poudre d'éjection et la substance support comme objet à heurter.

5. Procédé de traitement de surface d'un matériau métallique pulvérulent selon l'une quelconque des revendications 1 à 3, dans lequel le grenaillage est effectué en utilisant la substance support ayant une forme pulvérulente comme poudre d'éjection et le matériau métallique pulvérulent comme objet à heurter.

6. Procédé de traitement de surface d'un matériau métallique pulvérulent selon l'une quelconque des revendications 1 à 3, dans lequel la substance support se compose d'un matériau métallique pulvérulent du même matériau et du même diamètre de grain moyen que le matériau métallique pulvérulent, et la poudre d'éjection et l'objet à heurter sont tous deux transformés en matériau métallique pulvérulent.

7. Procédé de traitement de surface d'un matériau métallique pulvérulent selon l'une quelconque des revendications 1 à 5, dans lequel un matériau de la substance support est un métal ayant une dureté égale ou supérieure à la dureté du matériau métallique pulvérulent ou une céramique ayant une dureté égale ou supérieure à la dureté du matériau métallique pulvérulent après le traitement de surface.
